

# UNITED STATES PATENT OFFICE.

ARTHUR D. LITTLE, OF BROOKLINE, MASSACHUSETTS, ASSIGNOR TO ARTHUR D. LITTLE, INCORPORATED, OF BOSTON, MASSACHUSETTS, A CORPORATION OF MASSACHUSETTS.

## PAPER TOWEL.

1,122,959.

Specification of Letters Patent. Patented Dec. 29, 1914.

No Drawing.

Application filed September 23, 1912. Serial No. 721,922.

To all whom it may concern:

Be it known that I, ARTHUR D. LITTLE, a citizen of the United States, residing at Brookline, in the county of Norfolk and State of Massachusetts, have invented certain new and useful Improvements in Paper Towels, of which the following is a specification.

This invention relates to paper towels and similar articles, the object of the invention being to provide articles of this kind combining with the necessary highly bibulous or absorptive character, such degree of mechanical strength, even when wet, as is sufficient for their intended use.

Sanitary considerations, cheapness and convenience have led to many attempts to substitute paper for cloth as a material for towels, but in no case within my knowledge have the results been satisfactory. Unsized paper is sufficiently absorptive but is deficient in mechanical strength when wet. Sized paper, on the other hand, may have the necessary strength to withstand handling when wet, but is comparatively unab- sorbent, and is usually stiff and harsh to the touch when crumpled. If paper be lightly sized, it loses in absorptive capacity and softness in proportion as it gains in mechanical strength, with the result that under no conditions does it combine a high degree of absorptive capacity with adequate strength in the wet condition.

I have found that towels having a highly absorptive capacity combined with sufficient mechanical strength to endure handling even when practically saturated with moisture may be made as follows: A thin, highly flexible water leaf or unsized paper possessing the property of absorbing water promptly and in large amount, said paper being of the kind now commonly used for towels or napkins, is reinforced along relatively narrow and preferably connecting or intersecting lines, which lines bound areas of paper retaining unchanged or substantially unchanged its original absorptive capacity. The reinforcing lines may be varied in width, number and spacing to afford the necessary strength, and the thickness and texture of the paper may be selected to give the requisite absorptive capacity. By imprinting the reinforcing lines on crimped or crinkled papers, such as are commonly used for napkins or towels a material increase

in the absorptive surfaces bounded by these lines is secured.

The reinforcing lines may comprise films of water-resisting material printed, ruled or otherwise applied to the sheet, or completely or partially impregnating the sheet, the essential requirement being that the material shall possess sufficient strength, along the lines of reinforcement, to prevent the wet sheet from being reduced, under ordinary conditions of handling, to a pulpy mass as is the case with the untreated sheet. Or, as a modified embodiment of the invention, the lines of reinforcement may be produced in or from the structure of the paper itself, by treatment with appropriate modifying reagents. In either case, the size of the absorbent areas bounded by the reinforcing lines is in large part determined by the length of the fibers composing the sheet, it being desirable that a considerable proportion of the fibers within the absorbent area should be at some point in contact with the reinforcing substance, and held by it in place. For example, I have found absorbent areas three-sixteenths of an inch square to be satisfactory in case of ordinary cotton or sulfite papers, although considerable latitude in this respect is permissible. If desired, the lines may be of varying width, as for example a comparatively coarse reticulation of relatively wide and strong lines of reinforcement, the larger areas so formed being further subdivided by finer lines.

As examples of the first of the above-mentioned methods of treatment, I may apply a suitable reinforcing and water-resisting material by printing or analogous methods, the material being applied in a liquid or plastic state. The reinforcing material is usually structureless, and it is essential that it should be of such character that it is either substantially unaffected by short contact with water, or at least insures that the treated portions of the paper shall retain, when first moistened, sufficient strength to constitute a reinforcement under the conditions of use.

Because of its strength and cheapness, I prefer to use gelatin or glue as a reinforcing material, with or without the addition of glycerin. The glue may be conveniently applied to the paper by printing, ruling or otherwise, as for example in accordance with the methods used in printing calico, 110

along the intended lines of reinforcement or reticulation in the form of a thick solution in water, and thereafter rendered insoluble and sufficiently waterproof for the purposes 5 of my invention by treatment with formaldehyde either as a vapor or in solution. Such use of formaldehyde has the further advantage of sterilizing the towel. A solution of casein to which formaldehyde in 10 the proper proportion has been directly added may also be employed in place of the foregoing; or other plastics or adhesives may be substituted, as for example solutions or pastes of nitrocellulose or cellulose acetate. Or the paper may be printed 15 along the selected lines by a solution of rosin size, followed by a treatment with alum solution along the same lines; or other suitable sizing materials capable of affording 20 the necessary reinforcement may be employed.

It is obvious that the reinforcing material may be colored as desired for the production of special designs or artistic effects, and 25 that the arrangement of the lines of reinforcement or reticulation may be such as will produce or contribute to such effects. It is further obvious that the lines themselves need not be rectilinear or even continuous, nor need they bound completely 30 close areas so long as the reinforcing material is so distributed locally as to provide the requisite degree of strength in the towel as a whole when wet. 35 Examples of the second mode of treatment above mentioned consist in forming the reinforcing lines from the substance of the paper itself, as by printing on the water leaf paper with strong sulfuric acid or zinc chlorid solution in such manner as 40 locally to parchmentize the paper along the selected lines, and thereafter washing to remove the chemical.

While I prefer to use a true water leaf 45 paper for reinforcement as described, it is obvious that any paper of sufficient absorptive capacity and rapid rate of absorption may be substituted therefor, provided such paper is not objectionably stiff or harsh 50 in use.

In the reinforcement of thin, highly-flexible and absorptive papers of the character contemplated in accordance with this invention, no substantial or appreciable condensation of portions of the sheet occurs, so 55 that the finished towel is of substantially uniform thickness throughout and is substantially free from condensed lines or areas.

I claim:—

1. A towel or similar article consisting of a thin, highly-flexible sheet of absorptive paper, having a reinforcing-agent applied thereto along lines selected with reference to the reinforcement of the entire sheet, said 60 towel of substantially uniform thickness throughout and free from condensed portions.

2. A towel or similar article consisting of a thin, highly-flexible sheet of absorptive 70 paper, having a water-resisting reinforcing-agent applied thereto by printing or equivalent method along lines selected with reference to the reinforcement of the entire sheet, said towel of substantially uniform 75 thickness throughout and free from condensed portions.

3. A towel or similar article consisting of a thin, highly-flexible sheet of crinkled absorptive paper, having a reinforcing- 80 agent applied thereto along lines selected with reference to the reinforcement of the entire sheet, said towel of substantially uniform thickness throughout and free from condensed portions.

4. A towel or similar article consisting of a thin, highly-flexible sheet of crinkled absorptive paper, having a water-resisting reinforcing-agent applied thereto by printing or equivalent method along lines selected with reference to the reinforcement of the entire sheet, said towel of substantially uniform thickness throughout and free from condensed portions.

In testimony whereof I affix my signature 95 in presence of two witnesses.

ARTHUR D. LITTLE.

Witnesses:

JOHN G. CALLAN,  
HARRY S. MORK.